

March 3, 1964

D. S. POKRAS ET AL

3,123,484

ELECTROLESS GOLD PLATING SOLUTION

Filed Dec. 15, 1960

2 Sheets-Sheet 1

**FIG. I.** ELECTROLESS GOLD SOLUTION WITH CITRIC ACID BASE



Donald S. Pokras,  
Thomas L. Sullens,  
Robert F. Walton

BY  
*Stevens, Davis, Miller & Mosher*  
ATTORNEYS

March 3, 1964

D. S. POKRAS ET AL

3,123,484

ELECTROLESS GOLD PLATING SOLUTION

Filed Dec. 15, 1960

2 Sheets-Sheet 2

ELECTROLESS GOLD SOLUTION WITH TARTARIC ACID BASE

FIG. 2.



INVENTORS

Donald S. Pokras,  
Thomas L. Sullens,  
Robert F. Walton

BY

*Stevens, Davis, Miller & Mosher*  
ATTORNEYS

## 1

3,123,484

ELECTROLESS GOLD PLATING SOLUTION  
Donald S. Pekras, Thomas L. Sullens, and Robert F. Walton, Dallas, Tex., assignors to Texas Instruments Incorporated, Dallas, Tex., a corporation of Delaware  
Filed Dec. 15, 1960, Ser. No. 76,036  
4 Claims. (Cl. 106—1)

This invention relates to an improvement in the deposition of gold on a substrate. More specifically the invention relates to an improved electroless gold plating solution and to the method of preparing the same.

The three types of gold plating processes now available are electrolytic gold plating, the immersion process of gold plating and the electroless process of gold plating.

The electrolytic process of gold plating is carried out when the metal being plated transfers an electron to the gold anion, thus converting the gold anion to metallic gold at the metal surface and concurrently depositing the gold thereon. Any thickness of gold may be plated onto a metal surface by this process. One disadvantage of the electrolytic process is that the gold plating is not uniform over the surface of the metal body if the surface is irregular. This means that sharp points of the metal body will be plated more heavily than the rest of the body.

The immersion process of gold plating is carried on by a chemical process. Initially, a chemical in the gold plating solution prepares the surface of the metal in such a way that a gold layer can be deposited on the metal. However, after the first layer of gold is deposited on the metal, the process stops. This is because the chemical reaction can no longer take place since the gold has covered the base metal surface.

The electroless gold plating process is characterized by the fact that the amount of gold deposited on the metal is proportional to the time that the metal remains immersed in the plating solution. A continuous plating action in an electroless solution is made possible by the fact that a constituent thereof continuously activates the gold surface that has already been plated onto the base metal.

It is to the last-named type of plating process that this invention relates. In the past, various solutions have been proposed by which to effect electroless plating of gold. The various solutions proposed have been subject to one or more disadvantages, principal among which has been the inability to produce a plating of uniform thickness and/or substantial thickness. Another drawback to electroless gold plating solutions heretofore known is that they produce coarse grain platings. It is to overcome these disadvantages that the present invention was conceived. By means of the present invention, a method of preparing an electroless gold plating solution and a novel gold plating solution are provided whereby it is possible to conduct an electroless plating process to produce gold coatings having superior properties. By using the composition of the present invention experimental data shows that almost any uniform thickness of gold can be plated by the process and that the plating will be characterized by an exceptionally fine grain.

It is therefore an object of the present invention to provide an electroless gold plating solution with a constant deposition rate.

It is another object of the present invention to provide a method for the electroless deposition of gold onto a substrate of a less noble metal to any useful desired thickness.

It is still a further object of the present invention to provide a method of preparing an electrolessly gold plating solution for depositing gold onto a less noble metal substrate, whereby the deposited gold layer has a uni-

## 2

form thickness, a fine grain structure and a much greater thickness than heretofore attainable.

It is a feature of the present invention to provide an electroless gold plating solution containing an amino acid or water soluble salt thereof.

It is still another feature of the present invention to provide an electroless gold plating solution containing hydroxy dicarboxylic or hydroxy tricarboxylic acids and an amino acid or a water soluble salt thereof.

It is still a further feature of the present invention to provide an electroless gold plating solution wherein a tungsten compound is added as a grain refiner.

Other and further objects and features of the present invention will become evident from the following detailed description of the preferred mode for carrying out the invention.

The constituents of the gold plating solution are a water soluble gold salt, an acid from the general groupings of hydroxy dicarboxylic or hydroxy tricarboxylic acids and an amino acid or a water soluble salt of an amino acid.

In general, the above three components when properly mixed result in an acidified gold solution containing the novel ingredient, that is, an amino acid or a salt thereof, that promotes or stimulates the electroless process. Various theories have been proposed as to the action due to the addition of the salt of an amino acid, one being that it furnishes the electrons to reduce the gold at the metal being plated, thereby allowing continued deposition of gold to any desired thickness. For additional features two other important components may be added. The plating solution will more readily retain its desirable plating characteristics if a buffer solution is used to maintain the pH of the solution within a given range. The buffer prevents the pH of the solution from becoming relatively too basic. A solution of pH exceeding a maximum value results in the rate of deposition of the gold being retarded and in some cases ceasing altogether. Last, the addition of a grain refiner is, in many instances, desirable to give a closely-packed fine grain deposit.

The preceding indicates the general class of constituents necessary for an electroless gold plating solution. Preferred compounds, salts and acids of the general classes of constituents will indicate desired plating solutions. For example, potassium gold-cyanide  $[KAu(CN)_2]$  can be used to furnish the gold content of the solution. Theoretically, potassium-gold-cyanide contains 68.3 percent gold by weight although impurities may reduce the percent weight of gold to a lower value. Gold cyanide ( $AuCN$ ), sodium-gold-cyanide  $[NaAu(CN)_2]$  and gold compounds with the addition of potassium cyanides or gold cyanides can be used to furnish the gold content of the plating solution.

To obtain the desired plating action the plating solution must be at least acidic and buffered so that the solution does not exceed a given pH, thereby becoming too basic.

A mild organic acid such as citric acid or tartaric acid will render the solution acidic as desired. Other organic acids can be used although the two acids mentioned give a preferred quality. For example an acid from the general groupings of hydroxy dicarboxylic or hydroxy tricarboxylic acids will work.

In order to obtain a fine grain deposit of gold a tungsten compound is added as a grain refiner. It has been found that tungstic acid works very well as a grain refiner. Other compounds such as orthotungstic acid, tungsten oxide or tungsten dioxide will work. Such compounds as sodium tungstate and sodium paratungstate will suffice. Also, potassium tungstate, potassium paratungstate or potassium metatungstate can be included.

For a proper plating action the solution must be buffered to a given pH value. It has been found that the addition of phthalic acid monopotassium salt-sodium hydroxide

successfully buffers the solution to a pH between 5.0 and 6.0. Other buffering agents will work such as acetic acid-sodium acetate, buffering at a pH of 4.6, secondary sodium citrate, buffering at a pH of 5.0, potassium acid phosphate-disodium phosphate, buffering at a pH of 6.8 or potassium acid phosphate-sodium hydroxide, buffering at a pH of 6.8. The plating solution best performs at a pH value between 5.0 and 6.0. The preferred buffering agent is phthalic acid monopotassium salt-sodium hydroxide.

Finally, an amino acid or a water soluble salt of an amino acid is necessary to give the electroless plating characteristic instead of an immersion characteristic. The preferred agent used is a salt of an amino acid, the salt being N,N-diethylglycine sodium salt, although compounds such as N,N-diphenylglycine sodium salt, N,N-dimethylglycine sodium salt and N-phenylglycine potassium salt will work.

The plating solution is composed of four parts, and these parts are mixed according to the procedure set out, as will be shown later. The general procedure for mixing will be given although various percentages will be indicated subsequent to the mixing procedure. The approximate amounts of deionized water are given in the following procedure for a volume of one liter of solution. Although the percentages by weight of the constituents may be changed, the same amounts of deionized water are usually used.

*Solution A.*—The water soluble gold salt (preferably potassium gold cyanide) is dissolved in about 500 cc. of deionized water. Separately, an acid from one of the general groupings of hydroxy dicarboxylic acid or hydroxytricarboxylic acid is dissolved in about 250 cc. of deionized water, the acid preferably being tartaric acid or citric acid. The tartaric acid or citric acid solution is added to the potassium gold cyanide solution and mixed thoroughly. The acidified potassium gold cyanide is heated to about 140° F. and subsequently cooled to room temperature. Then the solution volume is increased to about 800 cc. with deionized water.

*Solution B.*—An alkali base (preferably sodium hydroxide) is dissolved in about 100 cc. of deionized water and cooled to room temperature. The cationic compound (preferably tungstic acid) is dissolved in the alkali base solution. To this solution is added the same carboxylic acid as added in solution A, in this case tartaric or citric acid. Deionized water is added until the solution volume is about 150 cc.

*Solution C.*—An alkali base is dissolved in about 35 cc. of deionized water-sodium hydroxide if also used in solution B. The other constituent of the buffering agent (preferably phthalic acid monopotassium salt) is dissolved in the above alkali base solution.

*Solution D.*—The amino acid or water soluble salt of an amino acid (preferably N,N-diethylglycine sodium salt) is dissolved in about 10 cc. of deionized water.

To combine these solutions it has been found that the following procedure gives best results. Solutions A and B are mixed and the pH adjusted with the same alkali base or acid previously used to a value of between 4.6 and 6.8. That is, if the pH is adjusted to a more acidic value, tartaric acid or citric acid is used, the one used being the same as previously used in solutions A and B. If the pH is adjusted to a more basic value, sodium hydroxide is used if it were used previously. The exact amount of these additives cannot be specified but must be added in a quantity to adjust the pH properly.

Solution C is added to the adjusted solution of A and B. Then solution D is added to the combination of solutions A, B, and C.

During the mixing process the sodium hydroxide serves three purposes. First, the grain refiner commonly used, for instance, tungstic acid, is not easily dissolved in an acid, but is more easily dissolved in a base such as sodium hydroxide. Secondly, the sodium hydroxide is one

component of the buffer solution. Thirdly, the pH of the plating solution can be adjusted by the addition of sodium hydroxide.

In order to show preferred embodiments of the present invention specific percentages of the various constituents will be given although variations of these percentages can be used to prepare solutions that will work to varying degrees of optimization without departing from the scope of the invention. For example, the gold cyanide may be from 7 to 28 grams per liter. The citric acid or tartaric acid may be from 5 to 60 grams per liter. The tungstic acid may be from 5 to 90 grams per liter. The ratio of potassium acid phthalic to sodium hydroxide may be 5.10 to 1 by weight in solution. The N,N-diethylglycine sodium salt may be from one-half to 15 grams per liter.

It has been found experimentally that only slight variations in results are obtained when comparing a solution containing citric acid and a solution containing tartaric acid. To illustrate, the optimum chemical compositions of two solutions, one containing tartaric acid and the other containing citric acid, are identical. Experimentally determined, the optimum chemical composition of electroless gold plating solutions are as follows:

| Concentration of—                     | Citric Acid<br>Solution in<br>grams/liter | Tartaric Acid<br>Solution in<br>grams/liter |
|---------------------------------------|-------------------------------------------|---------------------------------------------|
| Potassium Gold Cyanide.....           | 28                                        | 28                                          |
| Citric Acid.....                      | 60                                        | None                                        |
| Tartaric Acid.....                    | None                                      | 60                                          |
| Tungstic Acid.....                    | 45                                        | 45                                          |
| Sodium Hydroxide.....                 | 16                                        | 16                                          |
| N,N-Diethylglycine Sodium Salt.....   | 3.75                                      | 3.75                                        |
| Phthalic Acid Monopotassium Salt..... | 25                                        | 25                                          |

The pH of the above solution(s) is adjusted with citric acid or tartaric acid, or sodium hydroxide to have a pH value of 5.0 to 6.0.

To illustrate the results of using these solutions the following data show the amounts of gold deposited from a citric acid and a tartaric acid electroless gold solution when used to plate both kovar metal and nickel metal.

#### TEST RESULTS FROM CITRIC ACID BASE ELECTROLESS GOLD SOLUTION

| Immersion time<br>(Minutes) | Weight of Gold<br>Deposit (mg./<br>sq. in.) | Base Material |
|-----------------------------|---------------------------------------------|---------------|
| 5                           | 1.250                                       | Kovar         |
| 10                          | 1.486                                       | Kovar         |
| 15                          | 2.541                                       | Kovar         |
| 30                          | 2.709                                       | Kovar         |
| 60                          | 5.599                                       | Kovar         |
| 120                         | 8.099                                       | Kovar         |
| 240                         | 14.815                                      | Kovar         |
| 360                         | 20.273                                      | Kovar         |
| 5                           | 0.552                                       | Nickel        |
| 10                          | 1.600                                       | Nickel        |
| 15                          | 1.635                                       | Nickel        |
| 30                          | 2.973                                       | Nickel        |
| 60                          | 5.838                                       | Nickel        |
| 120                         | 6.983                                       | Nickel        |
| 240                         | 10.073                                      | Nickel        |
| 360                         | 17.993                                      | Nickel        |

#### TEST RESULTS FROM TARTARIC ACID BASE ELECTROLESS GOLD SOLUTION

| Immersion time<br>(Minutes) | Weight of Gold<br>Deposit (mg./<br>sq. in.) | Base Material |
|-----------------------------|---------------------------------------------|---------------|
| 5                           | 0.965                                       | Kovar         |
| 10                          | 1.204                                       | Kovar         |
| 15                          | 2.043                                       | Kovar         |
| 30                          | 3.150                                       | Kovar         |
| 60                          | 3.984                                       | Kovar         |
| 120                         | 11.998                                      | Kovar         |
| 240                         | 21.015                                      | Kovar         |
| 360                         | 17.131                                      | Kovar         |
| 5                           | 0.928                                       | Nickel        |
| 10                          | 1.243                                       | Nickel        |
| 15                          | 1.503                                       | Nickel        |
| 30                          | 3.115                                       | Nickel        |
| 60                          | 5.169                                       | Nickel        |
| 120                         | 7.328                                       | Nickel        |
| 240                         | 11.863                                      | Nickel        |
| 360                         | 14.775                                      | Nickel        |

FIGURE 1 shows a graph of weight of gold deposited in mg./sq. in. versus immersion time in minutes for the citric acid base solution when plated on Kovar and nickel. FIGURE 2 shows a similar graph for the tartaric acid base solution. Both graphs show curves of a linear nature with evidently no limit as to the amount of gold that can be plated onto a metal when immersed for a sufficient length of time. These results (characteristic of an electroless solution) are distinct when contrasted with the results obtained by using an immersion process.

Other examples of composition percentages that will work but do not deposit as much gold per unit of time are as follows:

| Concentration of—                     | Citric Acid<br>Solution in<br>grams/liter | Tartaric Acid<br>Solution in<br>grams/liter |
|---------------------------------------|-------------------------------------------|---------------------------------------------|
| Potassium Gold Cyanide.....           | 14                                        | 7                                           |
| Citric Acid.....                      | 15                                        | None                                        |
| Tartaric Acid.....                    | None                                      | 60                                          |
| Tungstic Acid.....                    | None                                      | 45                                          |
| Sodium Hydroxide.....                 | None                                      | 16                                          |
| N,N-Diethylglycine Sodium Salt.....   | 3.75                                      | 3.75                                        |
| Phthalic Acid Monopotassium Salt..... | 25                                        | 25                                          |

The pH of the above solution(s) is adjusted with citric acid or tartaric acid, or sodium hydroxide to have a pH value of 5.0 to 6.0.

In the above examples, the other specific compounds, salts and acids of the general classes of constituents listed supra could have been used. Also the percentage of each component used can be varied within limits. The procedure as set forth for mixing the components to form the solutions will remain substantially the same, however.

It is to be understood that, although the invention has been described with specific reference to particular embodiments thereof, it is not to be so limited since changes and alterations therein may be made which are within the full intended scope of this invention as defined by the appended claims.

What is claimed is:

1. An electroless gold plating solution comprising an admixture 7 to 28 grams per liter of potassium gold cyanide, 5 to 60 grams per liter of an organic acid selected from the group consisting of citric acid and tartaric acid, 5 to 90 grams per liter of tungstic acid, and a ratio of 5.10:1 by weight in solution of potassium acid phthalate to sodium hydroxide, and  $\frac{1}{2}$  to 15 grams per liter of N,N-diethylglycine sodium salt.
- 10 2. An electroless gold plating solution comprising an admixture of 28 grams per liter of potassium gold cyanide, 60 grams per liter of an organic acid selected from the group consisting of citric acid and tartaric acid, 45 grams per liter of tungstic acid, 16 grams per liter of sodium hydroxide, 25 grams per liter of phthalic acid monopotassium salt and 3.75 grams per liter of N,N-diethylglycine sodium salt.
- 15 3. An electroless gold plating solution comprising an admixture of 7 grams per liter of potassium gold cyanide, 60 grams per liter of tartaric acid, 45 grams per liter of tungstic acid, 16 grams per liter of sodium hydroxide, 25 grams per liter of phthalic acid monopotassium salt and 3.75 grams per liter of N,N-diethylglycine sodium salt.
- 20 4. An electroless gold plating solution comprising an admixture of 14 grams per liter of potassium gold cyanide, 15 grams per liter of citric acid, 16 grams per liter of sodium hydroxide, 25 grams per liter of phthalic acid monopotassium salt and 3.75 grams per liter of N,N-diethylglycine sodium salt.
- 25 5. An electroless gold plating solution comprising an admixture of 2,819,187 Gutzeit et al. ..... Jan. 7, 1958
- 30 35 6. An electroless gold plating solution comprising an admixture of 2,836,515 McNally et al. ..... May 27, 1958
7. An electroless gold plating solution comprising an admixture of 2,969,295 Crishal ..... Jan. 24, 1961
8. An electroless gold plating solution comprising an admixture of 2,976,181 Brookshire ..... Mar. 21, 1961

References Cited in the file of this patent

UNITED STATES PATENTS

- |              |                      |               |
|--------------|----------------------|---------------|
| 35 2,819,187 | Gutzeit et al. ..... | Jan. 7, 1958  |
| 2,836,515    | McNally et al. ..... | May 27, 1958  |
| 2,969,295    | Crishal .....        | Jan. 24, 1961 |
| 2,976,181    | Brookshire .....     | Mar. 21, 1961 |